# EUROPEAN PATENT SPECIFICATION

(11) **EP 2 840 152 B1**
(45) Date of publication and mention of the grant of the patent: **17.10.2018**
(21) Application number: 12878418.8
(22) Date of filing: 06.06.2012
(51) Int. Cl.: C21B 5/00, C22B 1/245

(54) **BLAST FURNACE OPERATION METHOD USING FERROCOKE**
BETRIEBSVERFAHREN FÜR EINEN VERBRENNUNGSOFEN MIT FERROCOKE
PROCÉDÉ DE CONDUITE DE HAUT FOURNEAU UTILISANT DU FERROCOKE

(43) Date of publication of application: 25.02.2015
(73) Proprietor: JFE Steel Corporation, Tokyo 100-0011 (JP)
(72) Inventor: SATO, Takeshi, Tokyo 100-0011 (JP); SUMI, Hiroyuki, Tokyo 100-0011 (JP); FUJIMOTO, Hidekazu, Tokyo 100-0011 (JP); ANYASHIKI, Takashi, Tokyo 100-0011 (JP); SATO, Hideaki, Tokyo 100-0011 (JP)
(74) Representative: Hoffmann Eitle
(86) International application number: PCT/JP2012/065056
(87) International publication number: WO 2013/183170

(56) References cited:
- EP-A1- 1 445 334
- EP-A1- 2 431 484
- EP-A1- 2 450 459
- JP-A- H08 134 517
- JP-A- S63 210 207
- JP-A- 2006 028 593
- JP-A- 2008 056 985
- JP-A- 2008 111 176
- JP-A- 2011 162 845

## Description

### Technical Field

The present invention relates to a method for operating a blast furnace using carbon iron composite produced by briquetting a mixture of coal and iron ore and carbonizing the briquetted material.

### Background Art

In order to decrease the reducing agent rate of a blast furnace, it is effective to use carbon iron composite as a blast furnace material and to utilize the effect of lowering the temperature of the thermal reserve zone in the blast furnace induced by the carbon iron composite (for example, see Patent Literature 1). Carbon iron composite produced by carbonizing a briquetted material prepared by briquetting a mixture of coal and iron ore has high reactivity, accelerates reduction of sintered ore, can decrease the thermal reserve zone temperature of the blast furnace since reduced iron ore is partly contained, and thus can decrease the reducing agent rate.

An example of a method for operating a blast furnace using carbon iron composite is disclosed in Patent Literature 1, in which ore and carbon iron composite are mixed and charged into a blast furnace.

Compared to conventional metallurgical coke produced by carbonizing coal in a coke oven or the like, carbon iron composite is characterized by its high reactivity with CO₂ gas shown in formula (a) below. Metallurgical coke is hereinafter referred to as "conventional coke" to distinguish from the carbon iron composite. The reaction of formula (a) is a reaction through which CO₂ generated by reduction of ore shown in formula (b) below is recycled into CO gas having a reducing ability.

CO₂ + C → 2CO ··· (a)

FeO + CO → Fe + CO₂ ··· (b)

Accordingly, when the reaction represented by formula (a) occurs rapidly in a region where the CO₂ gas concentration is increased through the reaction represented by formula (b), the CO₂ gas is recycled into CO gas having a reducing ability and the reduction of ore is accelerated.

The region with a high CO₂ gas concentration in the blast furnace is closely related to the gas distribution in the radius direction. Control of gas flow in a radius direction of a blast furnace is a critical operational item that affects permeability and reducing performance. Iron raw materials such as sintered ore, lump ore, and pellets have smaller grain size than the conventional coke produced in a chamber-type coke oven and become fused at high temperature; thus, permeation resistance is increased in a region where the amount of ore is large with respect to the amount of the conventional coke in the radius direction, namely, where the ore/coke amount ratio is high, thereby inhibiting gas flow. Accordingly, the gas flow in the radius direction is controlled by introducing a deviation in the ore/coke amount ratio in the radius direction. In the region where the ore/coke amount ratio is high, the ore/reducing gas amount ratio is increased. As a result, the proportion of CO gas in the furnace gas turning into CO₂ by the reaction represented by formula (b) is increased and the CO₂ gas concentration is increased. Iron raw materials such as sintered ore, lump ore, pellets, and the like are hereinafter referred to as "ore".

In the layer height direction within the ore layer formed each time the raw materials are charged, part of CO in the reducing gas ascending from below turns into CO₂ as a result of ore reduction; accordingly, the CO₂ concentration is higher in the upper layer if the radius position is the same (for example, refer to Non Patent Literature 1).

Selectively placing the carbon iron composite in the region with a high CO₂ concentration will accelerate gasification reaction of the carbon iron composite and improvements in reduction degree and a decrease in reducing agent rate can be expected as a result.

### Citation List

### Patent Literature

[PTL 1] Japanese Unexamined Patent Application Publication No. 2006-28594

### Non Patent Literature

[NPL 1] Zairyo to Purosesu [Materials and Processes] 13, 2000, p. 893

EP 2 450 459 A1 discloses a method for operating a blast furnace, comprising forming a coke layer and an ore layer in a blast furnace, in which the coke layer is formed of conventional coke; and the ore layer is formed of carbon iron composite, conventional coke and ore, wherein the ore layer comprises a first ore layer and a second ore lawyer that are charged in two batches, and in both of the first and second ore layers, the carbon iron composite, the conventional coke, and the ore are mixed together.

EP 2 431 484 A1 discloses a method for operating a blast furnace, comprising: charging the blast furnace with a charging material including iron ore, coke, and carbon iron composite; injecting gas into the blast furnace from a shaft portion of the blast furnace; and controlling injection temperature, injection rate, or/and vertical injection position of the gas depending on a top gas temperature of the blast furnace.

### Summary of Invention

### Technical Problem

In order to yield the high reactivity of the carbon iron composite, that is, in order to rapidly convert CO₂ gas into CO gas, during operation of a blast furnace using the carbon iron composite, it is considered preferable to distribute the carbon iron composite so that the concentration of the carbon iron composite is high in the region with a high CO₂ concentration.

The gas distribution in the radius direction of the blast furnace is generally controlled by adjusting the ore/coke amount ratio in the radius direction. The region where the ore/coke amount ratio is high corresponds to the region with a high CO₂ concentration. In the case where carbon iron composite is used by being mixed into the ore layer and the carbon iron composite is uniformly mixed in all parts of the ore layer, it is difficult to increase the carbon iron composite ratio in the region where the ore/coke amount ratio is high.

In the layer height direction within the ore layer formed each time the raw materials are charged, part of CO in the reducing gas ascending from below turns into CO₂ as a result of ore reduction and thus the CO₂ concentration is increased in the upper layer. However, in the case where the carbon iron composite is uniformly mixed in the ore layer, the concentration of the carbon iron composite is not particularly high in the region with a high CO₂ concentration.

Accordingly, an object of the present invention is to address such issues of the related art and provide a method for operating a blast furnace using carbon iron composite, with which, when carbon iron composite is mixed with ore and used in a blast furnace, the carbon iron composite's function of recycling CO₂ generated by ore reduction into CO gas having a reducing property can be more effectively yielded.

### Solution to Problem

The features of the present invention that address these issues are as follows:
(1) A method for operating a blast furnace using carbon iron composite by forming a coke layer and an ore layer in the blast furnace, the method including:
   dividing ore into a plurarity of batches including two or more batches and charging the ore into a blast furnace to form an ore layer;
   mixing the carbon iron composite into the ore layer of at least one batch in the ore layer formed by the plurality of batches; and
   no carbon iron composite being mixed into the ore layer of at least another batch,
      wherein
   the ore is charged so that positions where the plurality of batches are charged vary in a furnace radius direction and an ore layer thickness ratio defined by ore layer thickness/(ore layer thickness + coke layer thickness) is varied in the furnace radius direction, and the carbon iron composite is mixed into an ore layer of a batch that has a relatively large ore layer thickness ratio.
(2) The method for operating a blast furnace using the carbon iron composite according to (1), wherein the ore is divided into two or more batches in a height direction of the ore layer and charged, and no carbon iron composite is mixed into at least an ore layer of a batch located at the bottom.
(3) The method for operating a blast furnace using the carbon iron composite according to (1), wherein the ore is divided into two batches in a height direction of the ore layer and charged so as to form an ore layer positioned in an upper portion and an ore layer positioned in a lower portion, and no carbon iron composite is mixed into the ore layer positioned in the lower portion.
(4) The method for operating a blast furnace using the carbon iron composite according to (1), wherein the ore is divided into three batches in a height direction of the ore layer and charged so as to form an ore layer positioned in an upper portion, an ore layer positioned in a middle portion, and an ore layer positioned in a lower portion, and no carbon iron composite is mixed into the ore layer positioned in the lower portion.
(5) The method for operating a blast furnace using the carbon iron composite according to (1) or (2), wherein the carbon iron composite in the ore layer has a mixing ratio of 1% by mass or more relative to the ore.
(6) The method for operating a blast furnace using the carbon iron composite according to (5), wherein the mixing ratio is 1% by mass or more and 9% by mass or less.
(7) The method for operating a blast furnace using the carbon iron composite according to (1) or (2), wherein an iron content of the carbon iron composite is 5% to 40% by mass.
(8) The method for operating a blast furnace using the carbon iron composite according to (7), wherein the iron content of the carbon iron composite is 10% to 40% by mass. Advantageous Effects of Invention

According to the present invention, the concentration of the carbon iron composite can be increased in a blast furnace in a region where the CO₂ concentration is high, ore reduction can be accelerated through a gasification reaction of the carbon iron composite, and thus the reducing agent rate can be decreased.

### Brief Description of Drawings

[Fig. 1] Fig. 1A is a graph showing an ore layer thickness ratio in a radius direction in the case where the ore batch is divided into two in the radius direction and Fig. 1B is a schematic vertical sectional view of a blast furnace in which the ore layer thickness ratio is large in a middle portion.
[Fig. 2] Fig. 2A is a graph showing an ore layer thickness ratio in a radius direction in the case where the ore batch is divided into two in the radius direction and Fig. 2B is a schematic vertical sectional view of a blast furnace in which the ore layer thickness ratio is large in a peripheral portion.
[Fig. 3] Fig. 3A is a graph showing an ore layer thickness ratio in a radius direction in the case where the ore batch is divided into two in a layer height direction and Fig. 3B is a schematic vertical sectional view of a blast furnace.
[Fig. 4] Fig. 4 is a graph showing a relationship between the ratio of carbon iron composite used and the reduction degree of sintered ore.
[Fig. 5] Fig. 5 is a graph showing a relationship between the iron content in the carbon iron composite and the reaction start temperature.
[Fig. 6] Fig. 6A is a plan view and Fig. 6B is a front view schematically showing the shape of the carbon iron composite.

### Description of Embodiments

In a typical blast furnace operation, conventional coke and ore are alternately charged from the furnace top so that coke layers and ore layers are alternately stacked inside the furnace. One known method for forming an ore layer by charging ore into the furnace is charging ore in several divided batches. This is necessary in some cases due to the limited capacity of the furnace top banker and, in other cases, employed as the means for controlling the grain size distribution in the radius direction achieved by introducing grain radius deviations among batches, for example. In the present invention, in forming an ore layer, the ore charge is divided into several batches and the amount of the carbon iron composite mixed is varied among batches so as to control the carbon iron composite mixing ratio in the radius direction and the layer height direction and increase the carbon iron composite ratio at a particular position. As a result, it becomes possible to increase the carbon iron composite ratio in the region where the CO₂ concentration is high. In other words, a blast furnace operation method that uses carbon iron composite includes forming a coke layer and an ore layer, in which the ore layer is formed as a plurality of batches ore layer divided into two or batches, carbon iron composite is mixed into at least one batch of an ore layer in the plurality of batches ore layer but not into at least one different batch of an ore layer.

The position where the carbon iron composite ratio is to be increased is preferably a position where the ore layer thickness ratio (= ore layer thickness/(ore layer thickness + coke layer thickness)) is large. When the carbon iron composite ratio at the position in the blast furnace radius direction where the ore layer thickness ratio is large is increased, the carbon iron composite ratio in the region where the CO₂ concentration is high can be increased and the effect of mixing the carbon iron composite can be further enhanced. Accordingly, in an operation in which the ore layer thickness ratio is varied in the furnace radius direction, ore is charged so that the furnace radius direction position varies among the batches of the ore layers and a carbon composite is mixed into a batch of an ore layer at a furnace radius direction position where the ore layer thickness ratio is relatively large. When the plurality of batches are two batches, the carbon iron composite is mixed into the batch having a larger ore layer thickness ratio. When the plurality of batches are three or more batches, the carbon iron composite is mixed into at least the batch having the highest ore layer thickness ratio and no carbon iron composite is mixed into the batch having the lowest ore layer thickness ratio.

The position where the carbon iron composite ratio is to be increased is preferably an upper portion of the ore layer. Increasing the carbon iron composite ratio in the upper portion of the ore layer can increase the carbon iron composite ratio in the region having a high CO₂ concentration and the effect of mixing the carbon iron composite can be further enhanced. In such a case, operation is conducted so that the ore layer is divided into two or more batches in the height direction of the ore layer and no carbon iron composite is mixed into at least the ore layer of the batch located at the bottom. The carbon iron composite is preferably mixed into at least the ore layer of the batch located at the top.

In the description below, the present invention is described using specific examples with reference to Figs. 1 to 3 each showing the ore layer thickness ratio (= ore layer thickness/(ore layer thickness + coke layer thickness)) and layer structure in the radius direction.

Fig. 1 shows the case in which the ore layer thickness ratio in the middle portion is large. After forming a coke layer 1 in one batch, an ore layer 2 and an ore layer 3 divided into two batches are charged. Carbon iron composite is mixed into the batch of the ore layer 2 which is the first batch corresponding to a high-thickness-ratio portion so that the carbon iron composite can be selectively mixed into a portion in the radius direction where the ore layer thickness ratio is high.

Fig. 2 shows the case in which the ore layer thickness ratio in the peripheral portion is large. The carbon iron composite is mixed into the batch of an ore layer 5 which is the second batch corresponding to a high-thickness-ratio portion. As a result, the carbon iron composite can be selectively mixed into a portion in the radius direction where the ore layer thickness ratio is high.

In Fig. 3, the carbon iron composite is mixed into a batch of an ore layer 7 corresponding to the upper part of the entire ore layer and thus the carbon iron composite can be selectively mixed into the ore upper layer portion.

The above-described cases involve two-batch charging of the ore layer. Alternatively, the ore layer may be divided into three or more batches and the carbon iron composite may be mixed into only a particular batch or batches (one or more batches but the number of batches is at least 1 smaller than the total batch number) in order to selectively mix the carbon iron composite in a particular region.

The amount of the carbon iron composite to be mixed into the ore is discussed here. To 500 g of sintered ore serving as ore, conventional coke and carbon iron composite were mixed and the mixture was reacted in a CO:N₂ = 0.3:0.7 (volume ratio) atmosphere at 900°C for 3 hours. The results are shown in Fig. 4. The amount of the conventional coke mixed was 6% by mass. According to Fig. 4, when the amount of the carbon iron composite mixed with the ore is 1.0% by mass or more, the effect of increasing the sintered ore reduction degree is exhibited but the effect is saturated at about 9% by mass. Accordingly, the amount of the carbon iron composite mixed into the ore is preferably 1.0% by mass or more and 9% by mass or less.

Regarding the properties of the carbon iron composite, the reactivity with CO₂ gas is not high if the iron content in the carbon iron composite is small but the strength of the carbon iron composite is degraded if the iron content is excessively large, making the carbon iron composite unsuitable for the blast furnace charge. Fig. 5 shows the relationship between the iron content in the carbon iron composite and the start temperature of the reaction of the carbon iron composite with the CO₂-CO mixed gas. According to Fig. 5, along with the increase in the iron content in the carbon iron composite, the reactivity is improved and the reaction start temperature is decreased. A large effect is exhibited at the iron content of 5% by mass and onward and the effect is saturated at 40% by mass or higher. Accordingly, it can be deduced that the preferable iron content is 5% to 40% by mass and more. Thus, the iron content in the carbon iron composite is preferably 5% to 40% by mass and more preferably 10% to 40% by mass.

### [EXAMPLES]

A blast furnace operation test was conducted by applying the method of the present invention. The carbon iron composite used was manufactured by briquetting a mixture of coal and iron ore with a briquetting machine, charging the briquettes into a vertical shaft furnace, and performing carbonizing. The shape of the carbon iron composite is illustrated in Fig. 6. The upper diagram of Fig. 6 is a plan view and the lower diagram of Fig. 6 is a front view. The dimensions shown in Fig. 6 are A = 30 mm, B = 25 mm, C = 18 mm. The iron content in the carbon iron composite was 30% by mass. Sintered ore was used as the ore.

Charging of raw materials into the blast furnace was conducted as follows: First, a coke layer constituted only by conventional coke was formed and then the ore was charged in two batches as illustrated in Fig. 1. The average carbon iron composite amount mixed was 100 kg/t. In conducting operation, the same percentage of the carbon iron composite was mixed into each of the two ore batches in one case and, in another case, the carbon iron composite was mixed into one (ore layer 2) of the two ore batches only. For the purposes of comparison, operation was also conducted without mixing the carbon iron composite.

The results are shown in Table 1.

**[Table 1]**

| | | Case a | Case b | Case c |
|---|---|---|---|---|
| Carbon iron composite rate (including Fe) | kg/t | 0 | 100 | 100 |
| Carbon iron composite rate (excluding Fe) | kg/t | 0 | 70 | 70 |
| Conventional coke rate | kg/t | 352 | 249 | 246 |
| Pulverized coal rate | kg/t | 126 | 126 | 126 |
| Reducing agent rate | kg/t | 478 | 445 | 442 |
| Gas utilization ratio | % | 50.3 | 54.0 | 54.5 |
| Reference | | Comparative Example | Comparative Example | Example |

Case a is a comparative example where the carbon iron composite was not mixed into any of the ore layers 2 and 3 in the distribution control shown in Fig. 1. Case b is also a comparative example where the carbon iron composite was mixed into both the ore layers 2 and 3 in the distribution control shown in Fig. 1. Case c is an example of the present invention where the carbon iron composite was mixed into the ore layer 2 only in the distribution control shown in Fig. 1. Compared to Case a, the reducing agent rate is low in Case b and Case c where the carbon iron composite was used. The gas utilization rate was higher and the reducing agent rate was lower in Case c where the carbon iron composite was mixed into the ore layer 2 only than in Case b. This is presumably because selectively mixing the carbon iron composite into a portion with a high ore layer thickness ratio promoted gasification of the carbon iron composite and allowed the reduction of the ore to progress.

Next, the ore was divided into two batches and charged as illustrated in Fig. 2. As described above, the average amount of the carbon iron composite mixed was 100 kg/t. In conducting operation, the same percentage of the carbon iron composite was mixed into each of the two ore batches in one case and, in another case, the carbon iron composite was mixed into one of the two ore batches only. Operation was also conducted without mixing the carbon iron composite.

The results are shown in Table 2.

**[Table 2]**

| | | Case d | Case e | Case f |
|---|---|---|---|---|
| Carbon iron composite rate (including Fe) | kg/t | 0 | 100 | 100 |
| Carbon iron composite rate (excluding Fe) | kg/t | 0 | 70 | 70 |
| Conventional coke rate | kg/t | 354 | 251 | 248 |
| Pulverized coal rate | kg/t | 126 | 126 | 126 |
| Reducing agent rate | kg/t | 480 | 447 | 444 |
| Gas utilization ratio | % | 50.0 | 53.7 | 54.2 |
| Reference | | Comparative Example | Comparative Example | Example |

Case d is a comparative example where the carbon iron composite was not mixed into any of the ore layers 4 and 5 in the distribution control shown in Fig. 2. Case e is also a comparative example where the carbon iron composite was mixed into both the ore layers 4 and 5 in the distribution control shown in Fig. 2. Case f is an example of the present invention where the carbon iron composite was mixed into the ore layer 5 only in the distribution control shown in Fig. 2. Compared to Case d, the reducing agent rate is low in Case e and Case f where the carbon iron composite was used. The gas utilization rate was higher and the reducing agent rate was lower in Case f where the carbon iron composite was mixed into the ore layer 5 only than in Case e. This is presumably because selectively mixing the carbon iron composite into a portion with a high ore layer thickness ratio promoted gasification of the carbon iron composite and allowed the reduction of the ore to progress.

Next, the ore was divided into two batches and charged as illustrated in Fig. 3. As in the case described above, the average amount of the carbon iron composite mixed was 100 kg/t. In conducting operation, the same percentage of the carbon iron composite was mixed into each of the two ore batches in one case and, in another case, the carbon iron composite was mixed into one of the two ore batches only. Operation was also conducted without mixing the carbon iron composite.

The results are shown in Table 3.

**[Table 3]**

| | | Case g | Case h | Case i |
|---|---|---|---|---|
| Carbon iron composite rate (including Fe) | kg/t | 0 | 100 | 100 |
| Carbon iron composite rate (excluding Fe) | kg/t | 0 | 70 | 70 |
| Conventional coke rate | kg/t | 351 | 248 | 245 |
| Pulverized coal rate | kg/t | 126 | 126 | 126 |
| Reducing agent rate | kg/t | 477 | 444 | 441 |
| Gas utilization ratio | % | 50.4 | 54.1 | 54.6 |
| Reference | | Comparative Example | Comparative Example | Example |

Case g is a comparative example where the carbon iron composite was not mixed into any of the ore layers 6 and 7 in the distribution control shown in Fig. 3. Case h is also a comparative example where the carbon iron composite was mixed into both the ore layers 6 and 7 in the distribution control shown in Fig. 3. Case i is an example of the present invention where the carbon iron composite is mixed into the ore layer 7 only in the distribution control shown in Fig. 3. Compared to Case g, the reducing agent rate is low in Case h and Case i where the carbon iron composite was used. The gas utilization rate was higher and the reducing agent rate was lower in Case i where the carbon iron composite was mixed into the ore layer 7 only than in Case h. This is presumably because selectively mixing the carbon iron composite into an upper layer of the ore layer promoted gasification of the carbon iron composite and allowed the reduction of the ore to progress.

### Reference Signs List

- 1: coke layer constituted by conventional coke
- 2: ore layer (first batch)
- 3: ore layer (second batch)
- 4: ore layer (first batch)
- 5: ore layer (second batch)
- 6: ore layer (first batch)
- 7: ore layer (second batch)

## Claims

1. A method for operating a blast furnace using carbon iron composite by forming a coke layer and an ore layer in the blast furnace, the method comprising:
dividing ore into a plurality of batches including two or more batches and charging the ore into a blast furnace to form an ore layer,
mixing the carbon iron composite into the ore layer of at least one batch in the ore layer formed by the plurality of batches, and
no carbon iron composite being mixed into the ore layer of at least another batch, wherein
the ore is charged so that positions where the plurality of batches are charged vary in a furnace radius direction and an ore layer thickness ratio defined by ore layer thickness/(ore layer thickness + coke layer thickness) is varied in the furnace radius direction, and
the carbon iron composite is mixed into an ore layer of a batch that has a relatively large ore layer thickness ratio.

2. The method for operating a blast furnace using the carbon iron composite according to claim 1, wherein
the ore is divided into two or more batches in a height direction of the ore layer and charged, and
no carbon iron composite is mixed into at least an ore layer of a batch located at the bottom.

3. The method for operating a blast furnace using the carbon iron composite according to claim 1, wherein
the ore is divided into two batches in a height direction of the ore layer and charged so as to form an ore layer positioned in an upper portion and an ore layer positioned in a lower portion, and
no carbon iron composite is mixed into the ore layer positioned in the lower portion.

4. The method for operating a blast furnace using the carbon iron composite according to claim 1, wherein
the ore is divided into three batches in a height direction of the ore layer and charged so as to form an ore layer positioned in an upper portion, an ore layer positioned in a middle portion, and an ore layer positioned in a lower portion, and
no carbon iron composite is mixed into the ore layer positioned in the lower portion.

5. The method for operating a blast furnace using the carbon iron composite according to claim 1 or 2, wherein the carbon iron composite in the ore layer has a mixing ratio of 1% by mass or more relative to the ore.

6. The method for operating a blast furnace using the carbon iron composite according to claim 5, wherein the mixing ratio is 1% by mass or more and 9% by mass or less.

7. The method for operating a blast furnace using the carbon iron composite according to claim 1 or 2, wherein the iron contents of the carbon iron composite is 5% to 40% by mass.

8. The method for operating a blast furnace using the carbon iron composite according to claim 7, wherein the iron contents of the carbon iron composite is 10% to 40% by mass.

## Patentansprüche

1. Verfahren zum Betreiben eines Hochofens unter Verwendung von Kohlenstoff-Eisen-Komposit durch Bilden einer Koksschicht und einer Erzschicht in dem Hochofen, wobei das Verfahren umfasst:
Aufteilen von Erz in eine Mehrzahl von Chargen, die zwei oder mehr Chargen beinhaltet, und Chargieren des Erzes in einen Hochofen um eine Erzschicht zu bilden,
Mischen des Kohlenstoff-Eisen-Komposits in die Erzschicht von zumindest einer Charge in der Erzschicht, die durch die Mehrzahl von Chargen gebildet wurde, und
wobei kein Kohlenstoff-Eisen-Komposit in die Erzschicht von zumindest einer anderen Charge gemischt wird, wobei
das Erz derart chargiert wird, dass die Positionen, an denen die Mehrzahl von Chargen chargiert werden, in einer Ofenradiusrichtung variieren und ein Erzschichtdickenverhältnis, definiert durch Erzschichtdicke/(Erzschichtdicke + Koksschichtdicke) in der Ofenradiusrichtung variiert wird, und
das Kohlenstoff-Eisen-Komposit in eine Erzschicht einer Charge gemischt wird, die ein relativ großes Erzschichtdickenverhältnis aufweist.

2. Verfahren zum Betreiben eines Hochofens unter Verwendung des Kohlenstoff-Eisen-Komposits gemäß Anspruch 1, wobei
das Erz in zwei oder mehr Chargen in einer Höhenrichtung der Erzschicht aufgeteilt wird und chargiert wird, und
kein Kohlenstoff-Eisen-Komposit in zumindest eine Erzschicht einer Charge gemischt wird, die sich unten befindet.

3. Verfahren zum Betreiben eines Hochofens unter Verwendung des Kohlenstoff-Eisen-Komposits gemäß Anspruch 1, wobei
das Erz in zwei Chargen in einer Höhenrichtung der Erzschicht aufgeteilt wird und chargiert wird, so dass eine Erzschicht, die in einem oberen Abschnitt positioniert ist, und eine Erzschicht, die in einem unteren Abschnitt positioniert ist, gebildet werden und
kein Kohlenstoff-Eisen-Komposit in die Erzschicht gemischt wird, die in dem unteren Abschnitt positioniert ist.

4. Verfahren zum Betreiben eines Hochofens unter Verwendung des Kohlenstoff-Eisen-Komposits gemäß Anspruch 1, wobei
das Erz in drei Chargen in einer Höhenrichtung der Erzschicht aufgeteilt wird und chargiert wird, so dass eine Erzschicht, die in einem oberen Abschnitt positioniert ist, eine Erzschicht, die in einem mittleren Abschnitt positioniert ist, und eine Erzschicht, die in einem unteren Abschnitt positioniert ist, gebildet werden und
kein Kohlenstoff-Eisen-Komposit in die Erzschicht gemischt wird, die in dem unteren Abschnitt positioniert ist.

5. Verfahren zum Betreiben eines Hochofens unter Verwendung des Kohlenstoff-Eisen-Komposits gemäß Anspruch 1 oder 2, wobei das Kohlenstoff-Eisen-Komposit in der Erzschicht ein Mischungsverhältnis von 1% in Masse oder mehr relativ zu dem Erz aufweist.

6. Verfahren zum Betreiben eines Hochofens unter Verwendung des Kohlenstoff-Eisen-Komposits gemäß Anspruch 5, wobei das Mischungsverhältnis 1% in Masse oder mehr und 9% in Masse oder weniger beträgt.

7. Verfahren zum Betreiben eines Hochofens unter Verwendung des Kohlenstoff-Eisen-Komposits gemäß Anspruch 1 oder 2, wobei der Eisengehalt des Kohlenstoff-Eisen-Komposits 5% bis 40% in Masse beträgt.

8. Verfahren zum Betreiben eines Hochofens unter Verwendung des Kohlenstoff-Eisen-Komposits gemäß Anspruch 7, wobei der Eisengehalt des Kohlenstoff-Eisen-Komposits 10% bis 40% in Masse beträgt.

## Revendications

1. Procédé pour mettre en oeuvre un haut-fourneau en utilisant un composite carbone fer en formant une couche de coke et une couche de minerai dans le haut-fourneau, le procédé comprenant :
la division du minerai en une pluralité de lots incluant deux lots ou plus et le chargement du minerai dans un haut-fourneau pour former une couche de minerai,
le mélange du composite carbone fer dans la couche de minerai d'au moins un lot dans la couche de minerai formée par la pluralité de lots, et
aucun composite carbone fer n'étant mélangé dans la couche de minerai d'au moins un autre lot, dans lequel
le minerai est chargé de sorte que des positions où la pluralité de lots est chargée varient dans une direction de rayon de four et un rapport d'épaisseur de couche de minerai défini par l'épaisseur de couche de minerai / (l'épaisseur de couche de minerai + l'épaisseur de couche de coke) est varié dans la direction de rayon de four, et
le composite carbone fer est mélangé dans une couche de minerai d'un lot qui a un rapport d'épaisseur de couche de minerai relativement grand.

2. Procédé pour mettre en oeuvre un haut-fourneau en utilisant le composite carbone fer selon la revendication 1, dans lequel
le minerai est divisé en deux lots ou plus dans le sens de la hauteur de la couche de minerai et est chargé, et
aucun composite carbone fer n'est mélangé dans au moins une couche de minerai d'un lot situé au fond.

3. Procédé pour mettre en oeuvre un haut-fourneau en utilisant le composite carbone fer selon la revendication 1, dans lequel
le minerai est divisé en deux lots dans le sens de la hauteur de la couche de minerai et est chargé de façon à former une couche de minerai positionnée dans une portion supérieure et une couche de minerai positionnée dans une portion inférieure, et
aucun composite carbone fer n'est mélangé dans la couche de minerai positionnée dans la portion inférieure.

4. Procédé pour mettre en oeuvre un haut-fourneau en utilisant le composite carbone fer selon la revendication 1, dans lequel
le minerai est divisé en trois lots dans le sens de la hauteur de la couche de minerai et est chargé afin de former une couche de minerai positionnée dans une portion supérieure, une couche de minerai positionnée dans une portion intermédiaire et une couche de minerai positionnée dans une portion inférieure, et
aucun composite carbone fer n'est mélangé dans la couche de minerai positionnée dans la portion inférieure.

5. Procédé pour mettre en oeuvre un haut-fourneau en utilisant le composite carbone fer selon la revendication 1 ou 2, dans lequel le composite carbone fer dans la couche de minerai a un rapport de mélange de 1% en masse ou plus par rapport au minerai.

6. Procédé pour mettre en oeuvre un haut-fourneau en utilisant le composite carbone fer selon la revendication 5, dans lequel le rapport de mélange est de 1 % en masse ou plus et 9 % en masse ou moins.

7. Procédé pour mettre en oeuvre un haut-fourneau en utilisant le composite carbone fer selon la revendication 1 ou 2, dans lequel la teneur en fer du composite carbone fer est de 5 % à 40 % en masse.

8. Procédé pour mettre en oeuvre un haut-fourneau en utilisant le composite carbone fer selon la revendication 7, dans lequel la teneur en fer du composite carbone fer est de 10 % à 40 % en masse.
